



US010400394B2

(12) **United States Patent**  
Cowan et al.

(10) **Patent No.:** US 10,400,394 B2  
(45) **Date of Patent:** Sep. 3, 2019

(54) **METHOD FOR ENGINEERING FIBERS TO IMPROVE PAPER PRODUCTION**

(71) Applicant: **Pulmac Systems International, Inc.**, Williston, VT (US)

(72) Inventors: **Joffrey Dard Cowan**, South Burlington, VT (US); **Wavell Frederick Cowan**, Montpelier, VT (US); **Robert Joseph White**, Williston, VT (US)

(73) Assignee: **Pulmac Systems International, Inc.**, Williston, VT (US)

(\*) Notice: Subject to any disclaimer, the term of this patent is extended or adjusted under 35 U.S.C. 154(b) by 0 days.

(21) Appl. No.: **15/895,040**

(22) Filed: **Feb. 13, 2018**

(65) **Prior Publication Data**

US 2018/0291556 A1 Oct. 11, 2018

**Related U.S. Application Data**

(62) Division of application No. 15/242,501, filed on Aug. 20, 2016, now Pat. No. 10,041,209.

(60) Provisional application No. 62/208,355, filed on Aug. 21, 2015.

(51) **Int. Cl.**

**D21G 9/00** (2006.01)  
**D21D 1/20** (2006.01)  
**D21D 1/02** (2006.01)  
**D21D 5/24** (2006.01)

(52) **U.S. Cl.**

CPC ..... **D21G 9/0018** (2013.01); **D21D 1/02** (2013.01); **D21D 1/20** (2013.01); **D21D 5/24** (2013.01)

(58) **Field of Classification Search**

CPC ..... D21D 1/02; D21D 1/20; D21G 9/0018  
See application file for complete search history.

(56) **References Cited**

**U.S. PATENT DOCUMENTS**

|             |        |                |
|-------------|--------|----------------|
| 3,802,964 A | 4/1974 | Forgacs et al. |
| 3,873,416 A | 3/1975 | Forgacs et al. |
| 4,292,122 A | 9/1981 | Karnis et al.  |

(Continued)

**FOREIGN PATENT DOCUMENTS**

|    |                 |         |
|----|-----------------|---------|
| CN | 102242511 A     | 11/2011 |
| DE | 102006020215 A1 | 11/2007 |

(Continued)

**OTHER PUBLICATIONS**

Tappi, Consistency Measurement and Control in a Tissue Mill, 2011, PaperCon.

(Continued)

*Primary Examiner* — Anthony Calandra

(74) *Attorney, Agent, or Firm* — Thomas G. Ference

(57) **ABSTRACT**

A method for treating cellulosic fibers to improve paper, board and tissue quality; the method involves splitting fibers from feed pulp into an original portion containing original fibers and a refineable portion containing original fibers. The refineable portion is refined to create a refined portion containing refined fibers. Varying amounts of the original unrefined fibers and refined fibers are blended together to form a recombined slurry that is processed by a paper machine into an optimized paper product. A master control system and fiber measurement system are integrated with the overall system to regulate all processing.

**6 Claims, 19 Drawing Sheets**

System for Engineering Fibers  
to Improve Paper Production  
(20,20b)



| (56)                                                                                                                                                                                                                                                                                                                                                 | References Cited |                      |                       |                 |                      |
|------------------------------------------------------------------------------------------------------------------------------------------------------------------------------------------------------------------------------------------------------------------------------------------------------------------------------------------------------|------------------|----------------------|-----------------------|-----------------|----------------------|
| U.S. PATENT DOCUMENTS                                                                                                                                                                                                                                                                                                                                |                  |                      |                       |                 |                      |
| 4,342,618 A                                                                                                                                                                                                                                                                                                                                          | 8/1982           | Karnis et al.        | 2004/0011483 A1       | 1/2004          | Hautala et al.       |
| 4,514,257 A                                                                                                                                                                                                                                                                                                                                          | 4/1985           | Karlsson et al.      | 2006/0289140 A1       | 12/2006         | Park et al.          |
| 4,562,969 A                                                                                                                                                                                                                                                                                                                                          | 1/1986           | Lindahl              | 2008/0029232 A1       | 2/2008          | Wikdahl              |
| 4,609,432 A *                                                                                                                                                                                                                                                                                                                                        | 9/1986           | Brucato .....        | D21C 9/001<br>162/141 | 2009/0301674 A1 | 12/2009 Niinimaki    |
| 4,704,201 A                                                                                                                                                                                                                                                                                                                                          | 11/1987          | Keck et al.          | 2014/0057105 A1 *     | 2/2014          | Pande .....          |
| 4,776,926 A                                                                                                                                                                                                                                                                                                                                          | 10/1988          | Lindahl              |                       |                 | D21B 1/04<br>428/401 |
| 4,886,576 A                                                                                                                                                                                                                                                                                                                                          | 12/1989          | Sloan                | 2018/0092397 A1 *     | 4/2018          | Pesendorfer .....    |
| 4,892,619 A                                                                                                                                                                                                                                                                                                                                          | 1/1990           | Tistad               | 2018/0135246 A1       | 5/2018          | A24D 1/027           |
| 5,131,980 A                                                                                                                                                                                                                                                                                                                                          | 7/1992           | Chamlee et al.       |                       |                 | Crossley et al.      |
| 5,133,832 A                                                                                                                                                                                                                                                                                                                                          | 7/1992           | Gilkey               |                       |                 |                      |
| 6,361,650 B1                                                                                                                                                                                                                                                                                                                                         | 3/2002           | Danielsson et al.    |                       |                 |                      |
| 6,440,272 B1                                                                                                                                                                                                                                                                                                                                         | 8/2002           | Binder et al.        |                       |                 |                      |
| 6,491,792 B2                                                                                                                                                                                                                                                                                                                                         | 12/2002          | Shakespeare et al.   |                       |                 |                      |
| 6,517,680 B1                                                                                                                                                                                                                                                                                                                                         | 2/2003           | Fredlund et al.      |                       |                 |                      |
| 6,746,572 B2                                                                                                                                                                                                                                                                                                                                         | 6/2004           | Schwartz             |                       |                 |                      |
| 6,846,381 B2                                                                                                                                                                                                                                                                                                                                         | 1/2005           | Jussila et al.       |                       |                 |                      |
| 7,077,930 B2                                                                                                                                                                                                                                                                                                                                         | 7/2006           | Ammala et al.        |                       |                 |                      |
| 7,083,049 B2                                                                                                                                                                                                                                                                                                                                         | 8/2006           | Schabel              |                       |                 |                      |
| 7,289,210 B2                                                                                                                                                                                                                                                                                                                                         | 10/2007          | Jang                 |                       |                 |                      |
| 7,381,295 B2                                                                                                                                                                                                                                                                                                                                         | 6/2008           | Kokkonen             |                       |                 |                      |
| 7,407,563 B2                                                                                                                                                                                                                                                                                                                                         | 8/2008           | hietaniemi           |                       |                 |                      |
| 7,972,476 B2                                                                                                                                                                                                                                                                                                                                         | 7/2011           | Scherb et al.        |                       |                 |                      |
| 8,262,680 B2                                                                                                                                                                                                                                                                                                                                         | 9/2012           | Ring                 |                       |                 |                      |
| 8,679,293 B2                                                                                                                                                                                                                                                                                                                                         | 3/2014           | Ding et al.          |                       |                 |                      |
| 8,764,936 B2                                                                                                                                                                                                                                                                                                                                         | 7/2014           | Laurila-Lumme et al. |                       |                 |                      |
| 8,877,010 B2                                                                                                                                                                                                                                                                                                                                         | 11/2014          | Saren                |                       |                 |                      |
| 8,926,793 B2                                                                                                                                                                                                                                                                                                                                         | 1/2015           | Goto et al.          |                       |                 |                      |
| 9,039,272 B2                                                                                                                                                                                                                                                                                                                                         | 5/2015           | Karki                |                       |                 |                      |
| FOREIGN PATENT DOCUMENTS                                                                                                                                                                                                                                                                                                                             |                  |                      |                       |                 |                      |
| EP                                                                                                                                                                                                                                                                                                                                                   |                  | 1889971 A1           | 2/2008                |                 |                      |
| EP                                                                                                                                                                                                                                                                                                                                                   |                  | 2009176 A2           | 12/2008               |                 |                      |
| SU                                                                                                                                                                                                                                                                                                                                                   |                  | 444848 A1            | 9/1974                |                 |                      |
| WO                                                                                                                                                                                                                                                                                                                                                   |                  | 9107231 A1           | 5/1991                |                 |                      |
| WO                                                                                                                                                                                                                                                                                                                                                   |                  | 2006108508 A1        | 10/2006               |                 |                      |
| WO                                                                                                                                                                                                                                                                                                                                                   |                  | 200706318 A2         | 6/2007                |                 |                      |
| WO                                                                                                                                                                                                                                                                                                                                                   |                  | 2009000348 A1        | 12/2008               |                 |                      |
| WO                                                                                                                                                                                                                                                                                                                                                   |                  | 2009077001 A1        | 6/2009                |                 |                      |
| OTHER PUBLICATIONS                                                                                                                                                                                                                                                                                                                                   |                  |                      |                       |                 |                      |
| Smook, Handbook for Pulp and Paper Technologists, 1992, Angus Wilde Publications, 2nd Edition, Chapter 9.                                                                                                                                                                                                                                            |                  |                      |                       |                 |                      |
| Herbert Sixta "Handbook of Pulp", 2006 rozt, WILEY-VCH Verlag GmbH & Co. KGaA, Weinheim, ISBN 978-3-527-30999-3, "5.2.1.2 Fiber Fractionation by Screening", "6.6.1 Screening and Cleaning Efficiency", "7.1 General Principles", "7.2.5.3 Pressurized Reactors", 7.5.5.3 Effect of Pulp Consistency "11.3.2.3 Supramolecular Structure", fig. 4.24. |                  |                      |                       |                 |                      |
| * cited by examiner                                                                                                                                                                                                                                                                                                                                  |                  |                      |                       |                 |                      |

System for Engineering Fibers  
to Improve Paper Production  
(20, 20a)



Figure 1

## Fiber Fractionation System (34, 34a)



Figure 2a

## Fiber Fractionation System (34, 34b)



Figure 2b



Figure 3

## Fiber Fractionation



Thin Walled Fiber

Figure 4a



Thick Walled Fiber

Figure 4b

## Fiber Measurement



Fiber Wall Thickness Measurement with RGB Circular Polarized Light

Figure 5a



Fiber Wall Thickness Distribution of Fractionated Pulp

Figure 5b

## Fiber Refining



Figure 6a



Refined Fiber

Figure 6b

## Crill Measurement

$$\text{Crill Bonding Area} = \frac{\text{UV Absorption}}{\text{IR Absorption}}$$

Figure 7a

### Crill Bonding Area Before and After Refining



Figure 7b

## Fiber Measurement System

80

Figure 8

## Fractionation Maintenance System

110

Figure 9

## Vibration Spectra and Characteristic



Figure 10

## Vibration Analysis



Figure 11

## Static Fiber Processing Flow Example 1

Figure 12

**Dynamic Fiber Processing Flow**  
**Example 2**

| Step 1                               | Step 2                                         | Step 3                                     | Step 4                                     | Step 5                                     | Step 6                                                     | Step 7                                                  |
|--------------------------------------|------------------------------------------------|--------------------------------------------|--------------------------------------------|--------------------------------------------|------------------------------------------------------------|---------------------------------------------------------|
| Original Fibers/<br>Slurry           | Splitting<br>Slurry                            | Fractionation                              | Refinery                                   | Capacitance                                | Blending                                                   | Optimized<br>Fibers/<br>Slurry                          |
| Original Slurry<br><u>22</u><br>100% | Fractionable<br>Portion<br><u>26</u><br>45-55% | Heavies<br>Fraction <u>55</u>              | Refined<br>Portion <u>40</u>               | Refined<br>Portion <u>40</u>               | Refined<br>Fibers<br>(Heavies)<br><u>18d</u><br>13.5-16.5% | Refined Fibers<br>(Heavies)<br><u>18d</u><br>13.5-16.5% |
|                                      |                                                | Heavy<br>Fibers <u>18c</u><br>13.5-16.5%   | Refined<br>Fibers <u>18d</u><br>13.5-16.5% | Non-Refined<br>Portion <u>38</u>           | Non-Refined<br>Portion <u>38</u>                           | +<br>Light Fibers<br><u>18b</u><br>33.5-36.5%           |
|                                      |                                                | Lights<br>Fraction <u>53</u>               | Light<br>Fibers <u>18b</u><br>33.5-36.5%   | Light<br>Fibers <u>18b</u><br>33.5-36.5%   | Light<br>Fibers <u>18b</u><br>33.5-36.5%                   | +<br>Optimized<br>Slurry<br><u>39</u><br>100%           |
|                                      | Original<br>Portion<br><u>28</u><br>45-55%     | Original<br>Portion<br><u>28</u><br>45-55% | Original<br>Portion<br><u>28</u><br>45-55% | Original<br>Portion<br><u>28</u><br>45-55% | Original<br>Fibers<br><u>18a</u><br>45-55%                 |                                                         |

Figure 13

System for Engineering Fibers  
to Improve Paper Production  
(20, 20b)



Figure 14

## Static Fiber Processing Flow

### Example 3

| Step 1                               | Step 2                                | Step 3                                                        | Step 4                               | Step 5                                |
|--------------------------------------|---------------------------------------|---------------------------------------------------------------|--------------------------------------|---------------------------------------|
| Original Fibers/<br>Slurry           | Splitting<br>Slurry                   | Refinery                                                      | Blending                             | Optimized Fibers/<br>Slurry           |
| Original Slurry<br><u>22</u><br>100% | Refinable Portion<br><u>60</u><br>15% | Refined Portion <u>40</u><br>Refined Fibers <u>18d</u><br>15% | Refined Fibers<br><u>18d</u><br>15%  | Optimized Slurry<br><u>39</u><br>100% |
|                                      | Original Portion<br><u>28</u><br>85%  | Original Portion<br><u>28</u><br>85%                          | Original Fibers<br><u>18a</u><br>85% |                                       |

Figure 15

## Dynamic Fiber Processing Flow

### Example 4

| Step 1                               | Step 2                                   | Step 3                                                           | Step 4                                                           | Step 5                                  | Step 6                                |
|--------------------------------------|------------------------------------------|------------------------------------------------------------------|------------------------------------------------------------------|-----------------------------------------|---------------------------------------|
| Original Fibers/<br>Slurry           | Splitting<br>Slurry                      | Refinery                                                         | Capacitance                                                      | Blending                                | Optimized Fibers/<br>Slurry           |
| Original Slurry<br><u>22</u><br>100% | Refinable Portion<br><u>60</u><br>10-20% | Refined Portion <u>40</u><br>Refined Fibers <u>18d</u><br>10-20% | Refined Portion <u>40</u><br>Refined Fibers <u>18d</u><br>10-20% | Refined Fibers <u>18d</u><br>10-20%     | Optimized Slurry<br><u>39</u><br>100% |
|                                      | Original Portion<br><u>28</u><br>80-90%  | Original Portion<br><u>28</u><br>80-90%                          | Original Portion<br><u>28</u><br>80-90%                          | Original Fibers<br><u>18a</u><br>80-90% |                                       |

Figure 16

Exemplary Process Parameters  
Table 1

| System       | Samples | Fractionation  | % Mixtures |           | Refining<br>Revs (1000) |
|--------------|---------|----------------|------------|-----------|-------------------------|
|              |         |                | Feed       | Refined   |                         |
| 20a          | A       | Fractionated   | 85         | 15        | 5                       |
| 20a          | B       | Fractionated   | 85         | 15        | 10                      |
| 20a          | C       | Fractionated   | 70         | 30        | 3                       |
| 20a          | D       | Fractionated   | 70         | 30        | 4                       |
| 20a          | E       | Fractionated   | 70         | 30        | 5                       |
| 20b          | F       | Unfractionated | 75         | 25 (Feed) | 5                       |
| 20a          | G       | Fractionated   | 75         | 25        | 10                      |
| 20a          | H       | Fractionated   | 75         | 25        | 10                      |
| Conventional | I       | Unfractionated | -          | 100       | 0                       |
| Conventional | J       | Unfractionated | -          | 100       | 1                       |
| Conventional | K       | Unfractionated | -          | 100       | 2.5                     |
| Conventional | L       | Unfractionated | -          | 100       | 5                       |
| Conventional | M       | Unfractionated | -          | 100       | 7.5                     |

Figure 17

## Exemplary Paper Strength Using New System



Figure 18

## 1

METHOD FOR ENGINEERING FIBERS TO  
IMPROVE PAPER PRODUCTION

## RELATED APPLICATIONS

This application is a division of U.S. patent application Ser. No. 15/242,501, filed on Aug. 20, 2016 and entitled "System for Engineering Fibers to Improve Paper Production", which claims the benefit of priority of U.S. Provisional Patent Application No. 62/208,355, filed Aug. 21, 2015, both of which are herein incorporated by reference.

## FIELD

The present invention generally relates to a system for making paper from cellulosic fibers. More specifically, it relates to a system that engineers the cellulosic fibers to improve paper quality and reduce paper production costs.

## BACKGROUND

Paper, board and tissue are made from pulp that includes cellulosic fibers originally processed from wood chips. These chips are process mechanically or chemically to liberate the fibers from the fiber/lignin structure. Liberated fibers are usually bleached and refined as a single slurry before being formed and dried on a paper machine to make reels of paper. Softwood and hardwood fibers are usually processed separately until final blending just before paper machine processing.

Cellulosic fibers are a natural biological material derived from trees. As a biological material there is great diversity in fiber quality within one tree, let alone regionally and among different species. Current state of the art paper fabrication systems generally assume this diversity is a constant when transforming fibers into paper with the exception of distinguishing between softwood and hardwood fibers. In order to accommodate this assumption, large operating safety margins are built into the paper making process. The assumption that all incoming fiber quality is constant limits the potential benefit of specific fibers in the overall distribution and also limits the flexibility of optimization within the overall process. For example, if one tries to improve sheet strength through refining then water removal will be adversely affected and vice versa. The ability to change paper properties independent of paper machine operation variables is restricted by the assumption that pulp is made up of fibers with constant quality.

The present invention aims to provide a new system for treating cellulosic fibers that improves upon the currently unresolved issues described above by allowing one to select out defined fiber distributions that can be independently processed and recombined to make a superior paper product at lower costs.

## SUMMARY

In one implementation, the present disclosure is directed to a device for monitoring the interaction of fluid suspended cellulosic fibers being dynamically processed by a fractionator. The device is comprised of a vibration sensor and a vibration analyzer. The vibration sensor measures the vibration spectrum of the fractionator. The vibration analyzer determines vibration characteristics of the fractionator spectrum and compares the vibration characteristics to an acceptable characteristic; if the fractionator vibration characteristic is outside of a characteristic limit an alert signal is generated.

## 2

In another implementation, the present disclosure is directed to a system for measuring properties of fluid suspended cellulosic fibers. The system is comprised of a fractionator, a fractionator monitoring device and a vibration analyzer. The fractionator monitoring device includes a vibration sensor.

In another implementation, the present disclosure is directed to a system for engineering fiber properties of fluid suspended fibers, the fibers pass through primary, secondary, and/or tertiary fractionators to generate fractionated fiber slurries. Each fractionator has an incoming fractionable portion and produces a heavies fraction and a lights fraction. The system is comprised of an incoming fiber measurement device and a heavies fiber measurement device. The incoming fiber measurement device is interfaced to measure incoming fiber properties of the fractionable portion. The heavies fiber measurement device is interfaced to measure outgoing heavies fiber properties of a combination of the heavies fractions from the plurality of fractionators. Incoming fractionable fiber properties are compared to the combination of outgoing heavies fiber properties and a process parameter is adjusted to generate a targeted fiber property.

In yet another implementation, the present disclosure is directed to a system for engineering fiber properties of fluid suspended cellulosic fibers. The system is comprised of a plurality of fractionators that generate fractionated fiber slurries, each fractionator receiving an incoming fractionable portion with incoming fiber properties and incoming pressure and each fractionator producing a heavies fraction and a lights fraction. The heavies fraction having outgoing heavies fiber properties and an outgoing heavies pressure, flow and consistency. The lights fraction having outgoing lights fiber properties and an outgoing lights pressure, flow and consistency. The system also includes an incoming fiber measurement device interfaced to measure the incoming fiber properties of a combination of the incoming fractionable fiber portions. The system further includes a heavies fiber measurement device interfaced to measure outgoing heavies fiber properties of a combination of the heavies fractions from the plurality of fractionators. The incoming fiber properties are compared to the outgoing heavies fiber properties and the heavies pressure, flow or consistency is adjusted relative to the incoming pressure, flow or consistency to optimize the outgoing heavies fiber properties.

In yet another implementation, the present disclosure is directed to a system for engineering cellulosic fibers suspended in a fluid that has been split into an original portion and a fractionable portion. The system is comprised of a fractionator to fractionate the cellulosic fibers of the fractionable portion into a heavies fraction and a lights fraction. The system also comprises a refiner to refine the heavies fraction into a refined heavies fraction. The system further comprises a fiber property measurement system interfaced to measure cellulosic fiber properties of the cellulosic fibers.

Measured cellulosic fiber properties are then used to determine an amount of said refined heavies fraction to be recombined with the lights fraction and original portion to construct a recombined slurry.

In still another implementation, the present disclosure is directed to a system for engineering cellulosic fibers suspended in a fluid that has been split into an original portion and a refinable portion. The system is comprised of a refiner to refine the refinable portion into a refined portion. The system further comprises a fiber property measurement system interfaced to measure cellulosic fiber properties of the cellulosic fibers. Measured cellulosic fiber properties are then used to determine an amount of said refined portion to

be re-combined with the original portion to construct a recombined slurry that will produce an optimized paper product.

In still yet another implementation, the present disclosure is directed to a method of engineering cellulosic fibers. The method comprises first providing cellulosic fibers suspended in a fluid and a fractionator. The method then involves separating the cellulosic fibers into an original portion and a fractionable portion and introducing the fractionable portion of the cellulosic fibers into the fractionator. The method further involves separating the cellulosic fibers into a heavies fraction and a lights fraction and then refining the heavies fraction of cellulosic fibers into a refined heavies fraction to maximize bonding area. Finally the method involves recombining the refined fraction with at least one from the group consisting of the original portion and the lights fraction to create a recombined slurry.

#### BRIEF DESCRIPTION OF DRAWINGS

For the purposes of illustrating the invention, the drawings show aspects of one or more embodiments of the invention. However, it should be understood that the present invention is not limited to the precise arrangements and instrumentalities shown in the drawings, wherein:

FIG. 1 is a schematic diagram of one exemplary deployment of the system for engineering fibers to improve paper production;

FIG. 2a is a schematic diagram of one embodiment of the fiber fractionation system shown in FIG. 1;

FIG. 2b is a schematic diagram of an alternative embodiment of the fiber fractionation system shown in FIG. 2a, now having primary, secondary and tertiary fractionators;

FIG. 3 is a schematic view diagraming the internal working of a hydrocyclone fractionator used in the system of FIGS. 2a and 2b;

FIG. 4a is a schematic, sectional view of a thin walled cellulosic fiber before treatment by the system of FIG. 1;

FIG. 4b is a schematic, sectional view of a thick walled cellulosic fiber before treatment by the system of FIG. 1;

FIG. 5a is a diagram illustrating one technique for measuring fiber wall thickness of fibers processed by the system of FIG. 1;

FIG. 5b is a graph of exemplary fiber wall thickness distribution for pulp after processing through the fiber fractionation system of the system of FIG. 1;

FIG. 6a is a schematic, perspective view of an unrefined fiber before treatment by the system of FIG. 1;

FIG. 6b is a schematic, perspective view of the cellulosic fiber of FIG. 6a, after one possible treatment step to the fiber is completed as part of the system of FIG. 1;

FIG. 7a is a diagram illustrating one technique for measuring fiber crill for fibers processed by the system of FIG. 1;

FIG. 7b is a graph of exemplary crill properties for pulp before and after processing through the refiner of the system of FIG. 1;

FIG. 8 is a schematic diagram of the fiber measurement system of the system shown in FIG. 1;

FIG. 9 is a schematic diagram of the fractionation maintenance system of the system shown in FIG. 1;

FIG. 10 is a plot of vibration spectra and a specific vibration characteristic that may be measured from the vibration sensor shown in FIG. 9;

FIG. 11 is a flowchart of how the vibration spectra and vibration characteristic shown in FIG. 10 may be used to produce an alert in conjunction with the fractionation maintenance system of FIG. 9;

5 FIG. 12 is an exemplary process flow diagram for one embodiment of processing cellulosic fibers in conjunction with the system of FIG. 1;

10 FIG. 13 is an exemplary process flow diagram for another embodiment of processing cellulosic fibers in conjunction with the system of FIG. 1;

15 FIG. 14 is a schematic diagram of another exemplary deployment of the system for engineering fibers to improve paper production;

FIG. 15 is an exemplary process flow diagram for one 15 embodiment of processing cellulosic fibers in conjunction with the system of FIG. 14;

FIG. 16 is an exemplary process flow diagram for another embodiment of processing cellulosic fibers in conjunction with the system of FIG. 14;

20 FIG. 17 is a table indicating processing for several samples using the system shown in FIGS. 1 and 14 as compared to standard conventional processing; and

FIG. 18 is a plot of sample data from FIG. 17 comparing strength of paper prepared with the present invention against 25 paper prepared with standard whole pulp refinement.

#### DETAILED DESCRIPTION

The present invention embraces the biological variability 30 of cellulosic fibers 18 (a.k.a. fiber) found in wood and provides a system 20 that uses this fiber variability to improve paper production and allow for new paper products to be produced with improved quality and reduced production costs. The way in which system 20 accomplishes this is 35 by separating cellulosic fibers 18, then preferentially refining these separated fibers to a higher level of development than can now be achieved with the common practice where the full pulp flow is refined, and then blending back preferentially refined pulp to accommodate for fiber quality 40 variations in the original pulp. Instead of adjusting refining, which is the current state of the art; paper makers will adjust blending to balance production output with respect to the type of paper and quality of paper. The resulting pulp mixture can be used to produce paper with various desired 45 improved characteristics and reduced process costs.

System 20 for engineering fibers to improve paper quality is illustrated in FIGS. 1-18. Cellulosic fibers 18 created from wood are generally suspended in a fluid such as water during processing. Suspended fibers along with the suspension fluid 50 are generally known as a slurry. The slurry may also include additives such as defoamers, bonding agents, sizing agents, retention agents, drainage agents, fillers, enzymes, etc. System 20 (20a and 20b), FIGS. 1 and 14 comprises incoming fibers (a.k.a. original fibers 18a) as original slurry 22 55 obtained from a pulp source 24. In one embodiment, FIG. 20a, original slurry 22 (a.k.a. feed or feed pulp) is then split between a fractionable portion 26 and the remaining original portion 28. Remaining original portion 28 is directed to blender 30. Fractionable portion 26 is then processed by 60 fiber fractionation system 34. Here fibers 18 are separated by a given fiber property/characteristic, such as fiber wall thickness, fiber density, fiber size, etc. One fraction, unrefined portion 38, is sent to refiner 36 where fibers 18 are refined to be refined is sent to refiner 36 where fibers 18 are refined 65 to create a refined portion 40. Refined fibers 18d are held in storage tank 42. Varying amounts of refined portion 40, non-refined portion 38 and original portion 28 are then

blended together in blender 30 to produce optimized slurry 39 with optimal characteristics to be processed by paper machine 44 and create an optimized paper product 46. For example, the cellulosic fibers may have the same or increased bonding area with better drainage or the optimized cellulosic product may have increased strength while maintaining bulk, caliper and stiffness. Although the word "paper" is used as a modifier throughout this disclosure as in "paper machine" and also as an example of an end product that can be fabricated with system 20, it should be understood that the use of the word "paper" is meant to also include board, tissue and all other paper products.

Fiber fractionation system 34 may be any type of system that can separate cellulosic fibers 18 based on a fiber property. Fiber properties may include fiber wall thickness, fiber density, fiber size (length, width), fiber shape, amount of crill/nanofibrils (total, attached, unattached), fines content, etc. In one embodiment fiber fractionation system 34a is a bank of hydrocyclones 50 connected in parallel, FIG. 2a. In another embodiment fiber fractionation system 34b may include hydrocyclones 50 in series to create primary, secondary, and/or tertiary banks in series, FIG. 2b. In FIG. 2b arrows indicate direction of flow. Fractionators may also be screens, differential belt washers, flotation devices, etc. Hydrocyclones 50 each separate cellulosic fibers 18 based on at least one from the group including fiber wall thickness and fiber size. Connecting multiple hydrocyclones 50 in parallel allows for greater throughputs as each hydrocyclone can only process a limited flow rate.

Fiber fractionation system 34 (34a and 34b), FIGS. 2a and 2b, may have additional components that aid in the process of fractionation. For example, an incoming diluter 48 may be used to adjust the fluid content of the fractionable portion 26 of the slurry before it enters hydrocyclone bank 47. A lights thickener 49 may be used to adjust the fluid content of the lights fraction 53 exiting fiber fractionation system 34. A heavies thickener 51 may be used to adjust the fluid content of the heavies fraction 55 exiting fiber fractionation system 34. Additionally pressure meters, mass flow meters, and consistency meters may be integrated to measure pressure, flow and consistency of the slurry as it enters the fiber fractionation system at fiber fractionation system inlet 57 and exits as one or more of the fractionated portions 53 and/or 55 at either lights outlet 59 or heavies outlet 61. Consistency is defined as the percent solids content in a slurry. Incoming pressure meter 54 measures incoming pressure of fractionable portion 26 to all fractionators. Incoming flow meter 56 measures a combination of incoming flow rates of fractionable portion 26 flowing into all fractionators. Heavies pressure meter 58, if present, measures outgoing heavies pressure of the heavies fraction 55. Heavies flow meter 62, if present, measures a combination of outgoing flowing rates of the heavies fraction 55 flowing from all fractionators. Incoming consistency is measured by fiber measurement system 80 as a combination of incoming consistency of fractionable portion 26 flowing into all fractions. Lights pressure meter 64 measures outgoing lights pressure of the lights fraction 53. Lights flow meter 68 measures a combination of outgoing flow rates of the lights fraction 53 flowing from all fractionators. Lights consistency is measured as outgoing lights consistency of lights fraction 53. Incoming pressure and consistency, outgoing heavies pressure and outgoing lights pressure can be adjusted relative to each other to regulate flow rates and the degree of fractionation desired.

Each hydrocyclone 50 works as shown in FIG. 3. Incoming slurry is fed under pressure through fractionator inlet 70.

Fractionator inlet 70 is offset to one side of hydrocyclone 50. The slurry spins in a downward spiral towards the outer walls of hydrocyclone 50 as depicted by heavies flow arrow 72. Thicker, heavy fibers 18c drift outwards towards the walls of hydrocyclone 50 and exit through the bottom heavies fractionator outlet 74. Lighter fibers 18b and fines drift towards the center of hydrocyclone 50 and spin centrally upwards as depicted by lights flow arrow 75. Fines are defined as fiber components that can pass through a 200-10 mesh Bauer McNett screen. These lighter fibers 18b and fines spiral upward exiting through the top lights fractionator outlet 76.

In one embodiment fiber fractionation system 34 operates as follows. Each fractionator receives incoming fractionable portion with incoming fibers properties, incoming pressure, and incoming consistency. The fractionators then generates fractionated fibers slurries. Each fractionator produces a heavies fraction and a lights fraction. The heavies fraction has outgoing fiber properties, outgoing pressure and outgoing consistency. The lights fraction has outgoing lights fiber properties, outgoing lights pressure and outgoing lights consistency. An incoming fiber measurement device is interfaced to measure the incoming fiber properties of a combination of said incoming fractionable fiber portions. A heavies fiber measurement device may be interfaced to measure outgoing heavies fiber properties of a combination of the heavies fractions from the plurality of fractionators. The incoming fiber properties are compared to the outgoing heavies fiber properties and for example the heavies pressure is adjusted relative to the incoming pressure to optimize the outgoing heavies fiber properties and to control fractionation efficiency.

FIGS. 4a and 4b depict cross-sections of a thin walled, light fiber 18b (a.k.a. lights) and a thick walled, heavy fiber 18c (a.k.a. heavies). The thicker the wall of fiber 18, the more weight the fiber has and the more likely to exit the bottom heavies fractionator outlet 74. The thinner the wall of fiber 18, the less weight the fiber has and the more likely to exit top lights fractionator outlet 76. Fiber wall thickness 35 may be measured by red green blue (RGB) circular polarized light as shown in FIG. 5a and taught in U.S. Pat. No. 7,289,210, which is herein incorporated by reference. FIG. 5b shows exemplary data where fiber wall thickness has shifted after fractionation.

Refinement of fibers 18 can be used to modify fiber components contained within the slurry. Refining is the development of a fiber to generate more surface area through mechanical, chemical or biological processing. FIGS. 6a and 6b schematically show the fiber components of crill/nanofibrils 78, macrofibrils 79, fiber width 81 and fiber length 83 before and after refinement. Generally these cellulosic components are sized as follows: crill/nanofibrils 78 (having lengths of 0.1-1 micron), macrofibrils 79 (having lengths of 1-20 microns), fiber widths 81 (20-microns to 1-millimeter) and fiber lengths 83 (1-5 millimeters). Other engineering or refinement of fibers 18 may include deflaking, deshiving or fiberizing. A fiber property such as the amount of crill 78 (total, attached and unattached) determines the bonding surface area of fiber 18 and directly relates to the strength of the paper. A larger percentage of crill 78, both attached and unattached also affects the speed of drying of paper, board and tissue and can affect the amount of energy and time required to make the paper, board and tissue and adversely affecting paper production costs. A thick walled or heavy unrefined original fiber 18a in cross-section is depicted in FIG. 6a. After refinement through refiner 36, the refined fiber 18d in cross-section will be

deformed and have more crill 78 (total, attached and unattached) as shown in FIG. 6b. Crill (total, attached and unattached) is cellulosic material in the nanofibril size range and is measured by the ratio of UV light absorption to IR light absorption as shown in FIG. 7a and taught in U.S. Pat. No. 4,514,257, which is herein incorporated by reference. Light is projected through the cellulose fiber components and scatter is recorded. Crill is calculated by the relationship between the scatter generated by UV versus IR light, where UV light scatters the nanofibrils (crill). FIG. 7b shows representative crill bonding area data before and after refining.

Fiber measurement system 80, FIG. 8, includes one or more fiber measurement devices. Although many fiber measurement devices are shown with fiber quality tester 104 testing many properties of the fiber, it should be understood that only a select few of the fiber measurement devices and properties may actually be implemented in any system 20 depending on what the final paper product to be manufactured requires. Fiber measurement system 80 may include incoming fiber measurement device 82. Incoming fiber measurement device 82 is interfaced to measure incoming fiber properties of the fractionable portion 26 and includes an incoming sampler 84. Fiber sampled from incoming fiber sampler 84 is directed to sample prep 86. Fiber measurement system 80 may include heavy fiber measurement device 88. Heavy fiber measurement device 88 is interfaced to measure outgoing heavies fiber properties of a combination of the heavies fractions from a plurality of fractionators and includes a heavy fiber sampler 90. Fiber sampled from heavy fiber sampler 90 is directed to sample prep 86. Fiber measurement system 80 may include light fiber measurement device 92. Light fiber measurement device 92 includes a light fiber sampler 94. Fiber sampled from light fiber sampler 94 is directed to sample prep 86. Fiber measurement system 80 may include refined fiber measurement device 96. Refined fiber measurement device 96 includes a refined fiber sampler 98. Fiber sampled from refined fiber sampler 98 is directed to sample prep 86. Fiber measurement system 80 may include blended fiber measurement device 100. Blended fiber measurement device 100 includes a blended fiber sampler 102. Fiber sampled from blended fiber sampler 102 is directed to sample prep 86. Individual fiber samples prepared by sample prep 86 are then each tested for one or more fiber properties or slurry attributes such as fiber dimensions (length and width), fines content, fiber wall thickness, percent crill (total, attached, detached), freeness, consistency, pH, etc. Sample prep 86 and the tests that follow for each fiber property make up the fiber quality tester 104. A fiber data controller 106 is integrated with fiber quality tester 104 to send appropriate fiber data to master control system 108.

In one embodiment fiber measurement system 80 is used to compare incoming fractionable fiber properties to a combination of outgoing heavies properties and then use this result to adjust process parameters to achieve a targeted fiber property. In another embodiment fiber measurement system 80 is used to compare incoming fractionable fiber properties to a combination of outgoing lights properties and then use this result to adjust process parameters to achieve a targeted fiber property.

System 20 may include a fraction maintenance system 110, FIG. 9. Fraction maintenance system 110 includes a fractionator monitoring device 112 interfaced with one or more fractionators to monitor operation of the fractionator. When fractionating by weight of fibers the fractionator is preferably a hydrocyclone 50. Fractionator monitoring

device 112 includes a vibration sensor. The vibration sensor measures the vibration spectrum of the fractionator. One example of a vibration spectra showing a vibration characteristic indicating a blockage within a hydrocyclone is shown in FIG. 10. A vibration analyzer, FIG. 11, determines vibration characteristics of the fractionator vibration spectrum and compares the vibration characteristics to an acceptable characteristic in vibration measurement module 114. If the fractionator vibration characteristics are outside of a characteristic limit (a.k.a. threshold) an alert is signaled. Alert data 116 is transmitted to master control system 108.

Fiber data controller 104 receives fiber data and uses that data for overall control of system 20 through master control system 108. Master control system 108 adjusts incoming pressure, incoming consistency, outgoing heavies pressure and outgoing lights pressure to regulate flow rates and the degree of fractionation desired. Master control system 108 also regulates refiner 36 to refine heavies fraction 55 to the appropriate level of refining. Master control system 108 further regulates the amount of refined fiber stored in storage tank 42. Master control system 108 also regulates how original unrefined fiber 18a, refined fiber 18d and possibly additionally fractionated unrefined fiber is blended in blender 30 to produce an optimized slurry with optimal characteristics to be processed by paper machine 44 to create an optimized paper, board or tissue products 46. Master control system 108 also receives fractionator alert data 116 and sends out alerts to keep fiber fractionator system 34 in optimal working condition.

In one embodiment, system 20, 20a, is used in a static mode where the amount of fiber flowing through each portion of the system is a constant pre-determined amount. FIG. 12 illustrates step-by-step processing for such an embodiment showing the amount of fiber flow in each portion of system 20. When operating in this mode, previous experimental data is used to predetermine what the fiber flow will be through each portion of system 20. In step 1—100-percent of original fibers 18a suspended in a fluid enters the system as original slurry. Step 2—the slurry is split. 50-percent goes to fiber fractionation system 34 as fractionable portion 26 and the other 50-percent (original portion 28) is redirected to blender 30. Step 3—fractionation occurs. The fractionable portion 26 is introduced into the fractionators and is separated/fractionated by the fractionators into 15-percent heavy fibers 18c (heavies fraction 55) and 35-percent light fibers 18b (lights fraction 53). The 35-percent lights fraction is directed to blender 30. Step 4—refining fibers to maximize bonding area, the 15-percent of heavies fibers is directed to and processed by refiner 36. Step 5—blending the three fiber types: original fibers 18a, light fibers 18b and refined heavy fibers 18d are recombined and blended together. Step 6—the optimized slurry is achieved and sent to paper machine 44 to be turned into an optimized paper, board or tissue product 46. Percentages stated above are only for this one illustrative example; however these percentages should not be considered limiting and other percentages may be used.

In one embodiment system 20 is used in a dynamic mode where the amount of fiber flowing through each portion of the system is adjusted as measurements come in and are analyzed by master control system 108. FIG. 13 illustrates step-by-step processing for such an embodiment showing ranges for the amount of fiber flow in each portion of system 20 at any given time. In step 1—100-percent of original fibers 18a suspended in a fluid enters the system as original slurry. Step 2—the slurry is split within the given ranges depending on what type of paper is to be manufactured and

feedback information gathered in the rest of the process flow. For example, fiber in the range of 45-55 percent goes to fiber fractionation system **34** as fractionable portion **26** and the other 45-55 percent (original portion **28**) is redirected to blender **30**. Step **3**—fractionation occurs. The fractionable portion **26** is introduced into the fractionators and is separated/fractionated into 13.5-16.5 percent heavy fibers **18c** (heavies fraction **55**) and 33.5-36.5 percent light fibers **18b** (lights fraction **53**). The 33.5-36.5 percent lights fraction is directed to blender **30**. Step **4**—refining, the 13.5-16.5 percent of heavies is directed to and processed by refiner **36**. Step **5**—capacitance involves storing the fiber and then drawing upon the stored fibers as needed to mix the ideal fiber composition. Step **6**—blending the three fiber types: original fibers **18a**, light fibers **18b** and refined heavy fibers **18d** are recombined and blended together in any percentage that is required to produce the optimized slurry. Step **7**—the optimized slurry is achieved and sent to paper machine **44** to be turned into an optimized paper, board or tissue product **46**. Percentages stated above are only for this one illustrative example; however these percentages should not be considered limiting and other percentages may be used.

In an alternative embodiment, FIG. **14**, system **20**, **20a** has been modified to remove fiber fractionation system **34** and fractionator maintenance control system **110** giving a modified system as shown in system **20**, **20b**. In system **20b**, cellulosic fibers **18** are split into a refinable portion **60** and the remaining original portion **28** at feed splitter **118**. Remaining original portion **28** is directed to blender **30**. Fibers **18** from refinable portion **60** are then refined into refine portion **40**. Refined fibers **18d** are held in storage tank **42**. Varying amounts of refined portion **40** and original portion **28** are then blended together in blender **30** to produce optimized slurry **39** with optimal characteristics to be processed by paper machine **44** and create an optimized paper product **46**.

In one embodiment, system **20**, **20b** is used in a static mode where the amount of fiber flowing through each portion of the system is a constant pre-determined amount. FIG. **15** illustrates step-by-step processing for such an embodiment showing the amount of fiber flow in each portion of system **20**. When operating in this mode, previous experimental data is used to predetermine what the fiber flow will be through each portion of system **20**. In step **1**—100-percent of original fibers **18a** suspended in a fluid enters the system as original slurry. Step **2**—the slurry is split. 15-percent goes to refiner **36** as refinable portion **60** and the other 85-percent (original portion **28**) is redirected to blender **30**. Step **3**—refining fibers to maximize bonding area, the 15-percent of refinable fibers is directed to and processed by refiner **36**. Step **4**—blending the two fiber types: original fibers **18a** and refined fibers **18d** are recombined and blended together. Step **5**—the optimized slurry is achieved and sent to paper machine **44** to be turned into an optimized paper, board or tissue product **46**. Percentages stated above are only for this one illustrative example; however these percentages should not be considered limiting and other percentages may be used.

In one embodiment, system **20**, **20b** is used in a dynamic mode where the amount of fiber flowing through each portion of the system is adjusted as measurements come in and are analyzed by master control system **108**. FIG. **16** illustrates step-by-step processing for such an embodiment showing ranges for the amount of fiber flow in each portion of system **20** at any given time. In step **1**—100-percent of original fibers **18a** suspended in a fluid enters the system as

original slurry. Step **2**—the slurry is split within the given ranges depending on what type of paper is to be manufactured and feedback information gathered in the rest of the process flow. For example, fiber in the range of 10-20 percent goes to refiner **36** as a refinable portion **60** and the other 80-90 percent (original portion) is redirected to blender **30**. Step **3**—refining, the 10-20 percent of refinable portion is directed to and processed by refiner **36**. Step **4**—capacitance involves storing the fiber and then drawing upon the stored fibers as needed to mix the ideal fiber composition. Step **5**—blending the two fiber types: original fibers **18a** and refined fibers **18d** are recombined and blended together in any percentage that is required to produce the optimized slurry. Step **6**—the optimized slurry containing optimized fibers is achieved and sent to paper machine **44** to be turned into an optimized paper, board or tissue product **46**. Percentages stated above are only for this one illustrative example; however these percentages should not be considered limiting and other percentages may be used.

FIG. **17** (Table 1) lists data for samples prepared in accordance with system **20** (**20a**, **20b**) discussed in this disclosure and also for comparison samples that were prepared using standard conventional processing. Variables included whether fractionation occurred, the amount of feed and refined fibers combined, and the amount of refining the fibers were exposed to. For samples that were fractionated, a portion of feed slurry was fractionated at 0.5% TAPPI Standard T240 consistency. TAPPI® is a registered trademark of Technical Association of the Pulp and Paper Industry, Inc. Fractionated heavies were refined in a TAPPI standard T248 PFI mill at varying revolutions. Fractionated and refined heavies were blended back with feed slurry at varying percentages. TAPPI Standard T227 CSF drainage testing was performed on each blended slurry. TAPPI Standard T205 handsheets at 80 g/m<sup>2</sup> were generated. TAPPI Standard T822 Ring Crush Strength Testing was performed. For samples that were not fractionated (unfractionated), a portion of feed slurry was refined in a TAPPI standard T248 PFI mill at varying revolutions. Refined feed slurry was then blended back with unrefined feed slurry at 25%. TAPPI Standard T227 CSF drainage testing was performed on each blended slurry. TAPPI Standard T205 handsheets at 80 g/m<sup>2</sup> were generated. TAPPI Standard T822 Ring Crush Strength Testing was performed. For standard conventional processing, all feed slurry was refined in a TAPPI standard T248 PFI mill at varying revolutions. TAPPI Standard T227 CSF drainage testing was performed on each level of refining. TAPPI Standard T205 handsheets at 80 g/m<sup>2</sup> were generated from sample from each level of refining. TAPPI Standard T822 Ring Crush Strength Testing was performed on all handsheets.

FIG. **18** shows a plot of the exemplary data for paper strength of the samples of FIG. **17** using standard refining practices and those practices outlined in this disclosure by the current invention associated with system (**20**, **20a**, **20b**). Triangular data points on the line are strength numbers of handsheets made from pulp using standard conventional refining practices. Circular data points are handsheet strength numbers made from pulp where highly refined fibers were blended with feed pulp at different blend percentages and refining levels. Paper strength was significantly increased using the system and method proposed by the current invention. TAPPI Standard T220 “beater curves”, plotting strength of increasingly beaten pulp with freeness, were used to quantify the paper and board making strength potential for a given pulp sample. The comparison to be

## 11

observed in FIG. 18 is the strength of new engineered paper according to the present invention with the TAPPI standard process. Obtaining higher strength at lower drainage levels is desirable as the easier it is for water removal at target strength, the greater the productivity (by increased production levels and with lower fiber usage). FIG. 18 shows refining heavies such that once blended back with original portion there is a step change of 5-15 percent higher ring crush strength at a target freeness (proxy for paper machine drainage) than when all fibers are refined. Refining has diminishing returns where increasing bonding levels are compromised by the break down in fiber structure. For the currently engineered fibers is it critical that only a portion of the fiber is refined. In this way it is possible to maximize bonding levels on that portion without compromising water removal or fiber structure. This is achieved in two ways, either by refining a portion of fractionated heavies or by refining a portion of the feed pulp. To get results A to H, which represents an average of 10% increase in strength at the same drainage as standard results, it is critical to blend either refined feed or refined fractionated heavies with feed pulp. These results cannot be achieved by conventionally refining of all feed pulp.

The advantages of system 20 is that instead of processing the fibers as a whole, a small portion of fibers with a specific fiber property can be separated out and only that fraction engineered by a mechanical or chemical process. For system 20a, three types of fibers (original, fractionated refined and fractionated non-refined) created by the system are then combined to create an optimum slurry to create optimized paper product 46. For system 20b two types of fibers (original and unfractionated refined) created by the system are then combined to create an optimum slurry to create optimized paper product 46. Cost savings are realized because only a small portion of the fibers have to go through special processing, e.g. refining to increase crill 78 (total, attached and unattached). Cost savings may also be realized as the final slurry may be optimized for drying and therefore require less time and energy to make optimized paper product 46. System 20 also has the advantage that a wide variety of specialty paper-products can be easily manufactured by having master control system 108 adjust fiber types and fiber amounts in situ as the paper mill adjust to different orders. Another advantage of the system 20 is that operating variance can be compensated with only blending changes and not both blending and refining changes. Still another advantage is that system 20 can reside in the pulp mill thus enhancing communication between pulp and paper machine personnel and minimizing paper machine personnel craft decision making.

While several embodiments of the invention, together with modifications thereof, have been described in detail herein and illustrated in the accompanying drawings, it will

## 12

be evident that various further modifications are possible without departing from the scope of the invention. The scope of the claims should not be limited by the preferred embodiments set forth in the examples, but should be given the broadest interpretation consistent with the description as a whole.

What is claimed is:

1. A method for engineering cellulosic fibers, comprising:
  - a) providing a system for engineering cellulosic fibers suspended in a fluid, the system including i) a feed splitter that splits fibers from feed pulp into an original portion containing original fibers and a refineable portion containing original fibers, ii) a fiber measurement system, iii) a refiner, iv) a storage tank for holding a refined portion from the refiner, v) a blender, and vi) a paper machine;
  - b) measuring original fiber quality variations of fiber properties in the original fibers;
  - c) splitting the original portion and the refineable portion at the feed splitter, wherein the original portion and the refineable portion have substantially the same composition after splitting;
  - d) refining the refineable portion through the refiner to create the refined portion containing refined fibers, the refined fibers refined to targeted refined fiber properties controlled by measurement, wherein the measurement occurs after refining;
  - e) recombining in the blender an amount of the refined portion with the original portion to create a recombined slurry;
  - f) adjusting the amount of refined portion coming from the storage tank that is recombined with the original portion to compensate for the original fiber quality variations of fiber properties in the original portion; and
  - e) making in the paper machine a paper product.
2. The method as recited in claim 1, wherein fiber quality variations are at least one from the group consisting of fiber length, fiber width, fines content, fiber wall thickness, percent crill attached, percent crill unattached and freeness.
3. The method as recited in claim 1, wherein the refineable portion is 10-25 percent of the original portion.
4. The method as recited in claim 1, wherein the paper product has a ring crush strength improvement at a target freeness than when all incoming fibers are refined together.
5. The method as recited in claim 1, further comprising adjusting the amount of refined portion from the storage tank that is recombined with the original portion to compensate for ring crush strength and water removal.
6. The method as recited in claim 1, further comprising adjusting the amount of refined portion from the storage tank that is recombined with the original portion to achieve different types of paper products from the same feed pulp.

\* \* \* \* \*